

# UNITED STATES PATENT OFFICE.

EUGÈNE SCHNEIDER, OF LE CREUSOT, FRANCE.

## ALLOY FOR ARMOR-PLATES AND OTHER USES.

No. 925,659.

Specification of Letters Patent.

Patented June 22, 1909.

Application filed August 2, 1907. Serial No. 386,834.

*To all whom it may concern:*

Be it known that I, EUGÈNE SCHNEIDER, citizen of the Republic of France, residing at Le Creusot, Saône-et-Loire, France, have 5 invented certain new and useful Improvements in Alloys for Armor-Plates and other Uses, of which the following is a specification.

The cementation of armor plates has resulted in considerably increasing the resistance offered to projectiles relatively to that obtaining with the homogeneous armor plates previously employed; so that recourse is now always had to cemented armor 15 plates hardened by different processes, for the purpose of opposing the passage of projectiles at high velocities and effecting their fracture by shock upon the impact face of such plates. Although presenting great resistance to uncapped projectiles, cemented armor plates offer but a relatively small resistance and one which is far from uniform when they are attacked by capped projectiles; in this case they present little superiority over uncemented plates of equal thickness.

The present invention relates to alloys by means of which it is possible to form homogeneous armor plates giving results 30 superior to those obtained with cemented plates. The homogeneous armor plates manufactured with these alloys present a more uniform resistance to the attack of uncapped projectiles and they also offer 35 greater resistance to capped projectiles than the best armor plates heretofore known.

The improved alloys are constituted in the following manner:—A steel comprising, in addition to the iron, per hundred parts:

|           |                 |
|-----------|-----------------|
| Carbon    | 0.30 to 0.50    |
| Manganese | less than 0.350 |
| Nickel    | 3 to 5          |
| Chromium  | 0.5 to 1.5      |

45 and while the metal is in fusion from 0.5 to 1.5% of molybdenum or 1 to 3% of tungsten, or again, 0.2 to 0.5% of vanadium are added thereto.

Instead of adding one only of the metals 50 indicated above to the steel separately, two may be added simultaneously; for example molybdenum and tungsten together, or molybdenum and vanadium, or tungsten and

vanadium. The three metals, tungsten, molybdenum and vanadium, may also be added 55 simultaneously. In these latter cases the proportions of the metals added to the steel are reduced in a proportionate manner as regards each of them.

The composition of the steel, indicated 60 above, is that which gives the best results in practice, but it is nevertheless capable of slight modifications.

The alloys constituted in the manner herein described present special properties 65 due to their homogeneity and to the presence in the initial steel of the molybdenum, tungsten or vanadium separately or combined in twos, or all three added together. The presence of the molybdenum, tungsten 70 or vanadium separately or combined in twos or all three added together to the nickel and chromium in the steel, advantageously replaces the high percentage of carbon in the impact face of cemented armor plates, because it makes it possible by any convenient 75 process of tempering to obtain in regard to this face, a hardness sufficient to crush the projectiles and preserve all the desirable malleability in the metallic mass for avoiding cracking on firing.

With the alloys indicated above, homogeneous armor plates may be manufactured without any cementation or addition of special bodies to one face, while at the same 85 time obtaining the proper qualities for resisting the attacks of capped and uncapped projectiles without cracking or scaling, in a more satisfactory manner than the armor plates hitherto known; this improvement is 90 particularly noticeable in the case of the capped projectiles which are employed in all navies.

Apart from the manufacture of armor plates, the herein described alloys are capable of numerous uses precisely owing to their homogeneity and their great resistance.

What I claim is:—

1. A steel alloy for armor plates containing carbon 0.3 to 0.5 per cent., manganese 100 not over 0.35 per cent., nickel 3 to 5 per cent.; chromium 0.5 to 1.5 per cent., molybdenum 0.5 to 1.5 per cent., and the remainder of iron.

2. A steel alloy for armor plates containing in one hundred parts, in addition to iron, 105 carbon 0.3 to 0.5, manganese less than 0.35,

nickel 3 to 5, chromium 0.5 to 1.5, molybdenum less than 1.5 and tungsten less than 3.

3. A steel alloy for armor plates containing carbon 0.3 to 0.5 per cent., manganese less than 0.35 per cent., nickel 3 to 5 per cent., chromium 0.5 to 1.5 per cent., tungsten less than 3 per cent., and the remainder of iron.

In testimony whereof I have affixed my signature in presence of two witnesses.

EUGÈNE SCHNEIDER.

Witnesses:

H. C. COXE,

CHARLES DE LAGRANGE.